

June 30, 1964

R. A. HEMSTOCK  
RECOVERY OF BITUMEN FROM TAR SANDS  
UTILIZING AN EVACUATION STEP  
Filed Oct. 6, 1961

3,139,397



Russell A. Hemstock Inventor

By *W.O. Tschelman*

Patent Attorney

# United States Patent Office

3,139,397

Patented June 30, 1964

1

3,139,397

## RECOVERY OF BITUMEN FROM TAR SANDS UTILIZING AN EVACUATION STEP

Russell A. Hemstock, Calgary, Alberta, Canada, assignor to Esso Research and Engineering Company, a corporation of Delaware

Filed Oct. 6, 1961, Ser. No. 143,404  
5 Claims. (Cl. 208—11)

The present invention is broadly concerned with the efficient recovery of hydrocarbons from tar sands. The invention is more particularly concerned with an improved technique of efficiently removing hydrocarbons, such as bitumen, tars, and the like, from tar sands containing the same, utilizing a particular technique involving a vacuum separation step. The present invention is more particularly concerned with the efficient recovery of hydrocarbons from tar sands such as Athabasca tar sands.

In various areas of the world, tar sands exist which contain various types of hydrocarbons as, for example, the heavy deposits of Athabasca tar sands existing in Canada. These sands contain tremendous reserves of hydrocarbon constituents. For example, the oil in the sands may vary from about 5% to 21% by weight, generally in the range of about 12% by weight. The gravity of the oil ranges from about 6° to 10° API, generally about 8° API. These sands may lie from zero to several hundred feet below an overburden and the beds may range from about 100 to 400 feet thick. A typical oil recovered from the sands has an initial boiling point of about 300° F., 1.0% distilled to 430° F., 20.0% distilled to 650° F. and 50.0% distilled to 980° F. However, the recovery of hydrocarbons in the past has not been effective to any great extent due to the deficiencies in operating techniques for the recovery of these hydrocarbons. For example, a relatively small amount of clay (from about 0% to 30%, usually about 5%) in the sand greatly retards recovery of the oil utilizing conventional water techniques. Apparently the oil and the clay from skins which envelop small pockets of water often containing finely divided sand; then the enveloped pockets are distributed in water, thus forming a type of emulsion.

Numerous attempts have been made in the past to recover bitumen from the Athabasca tar sands in various manners. For example, it has been suggested that a solvent be added in order to reduce the viscosity of the bitumen, and in conjunction with water, to float the bitumen solvent mixture away from the sand. Although this technique achieves a good separation of clean sand, the addition of water results in problems with the formation of stable emulsions and sludges which have been very difficult to separate. Thus, extensive supplementary processing has been required in order to avoid large oil losses.

It has also been suggested in the past that tar sands as they are mined be handled by a thermal process in order to recover the bitumen therefrom. However, this process has been uneconomical due to the large amount of heat which is lost due to the fact that the heat is imparted to the sand and cannot be effectively and efficiently recovered therefrom. It has been suggested for example that tar sands be handled in a direct fluid coking operation. However, as pointed out, this process is uneconomical for the reasons given above. Also, any process that will effectively handle tar sands must have the ability to handle a very wide range of tar sand and compositions which occur even in an immediate location. Some processes as, for example, direct fluid coking are able to handle these widely different compositions and, in accordance with the present process, employing a two-phase operation wherein in an initial phase a substantially richened tar sand is produced and wherein in the second phase the enriched sand is for example handled in a fluid coker, surprisingly effective results are secured.

2

The present invention may be readily understood by reference to the drawing illustrating one embodiment of the same. Referring specifically to the drawing, tar sands as mined are introduced into a shearing-mixing stage 1 by means of feed line 2. Water is introduced into line 2 and mixed with the sands by means of line 3. The water may be introduced directly into mixing-shearing zone 1. It is also to be understood that, while only one mixing zone is illustrated, a plurality of shearing-mixing zones may be used and a plurality of injection points also utilized.

The mixing operation in zone 1 is carried out under conditions wherein a shearing thrust is imparted to the sands being mixed with the added water. Under these conditions, substantially oil-free sands separate and the entire mixture is then passed into a second stage or zone 5 by means of line 4. In accordance with the present invention, additional water is introduced into zone 5 by means of line 6 while the zone is maintained under a vacuum by means of line 7. Under these conditions, sand and water separate and fall to the bottom and are removed by means of line 8. An oil phase forms in the upper area of zone 5, which phase is removed by means of line 9. It is preferred that the total amount of water added in the present process be in the range from about 40 to 400% of water, preferably in the range from about 50 to 150% of water by weight based upon the tar sands being processed and that the preferred temperature be about 50 to 90° F.

The process of the present invention may be more fully understood by the following examples illustrating the same.

### EXAMPLE 1

A 100 g. of a sample of tar sands (dry basis) containing 7 wt. percent connate water and 13 wt. percent oil was mixed with 30 wt. percent water for half a minute to effect disintegration of the tar sands into sand and very small oil particles distributed in water. This was carried out at 45° F. The mixture was transferred to a flask containing excess water and the pressure was reduced. When the pressure reached 200 mm. of mercury, oil floated to the surface. At lower pressure, increasing amounts of oil floated to the surface. Complete separation was obtained, with clean sand remaining at the bottom of the vessel, in less than half a minute from starting the evacuation.

It was observed that the very small oil particles that floated to the water surface immediately coalesced, forming large agglomerates, hence reducing the water content of the oil mass. These large oil agglomerates were skimmed off the surface of the water.

### EXAMPLE 2

The sand reduction in this operation can be compared with that from mixing with water and mechanical separation. This is shown in the following table:

Table I

GOOD SAND REDUCTION IS ACCOMPLISHED AT LOWER TEMPERATURES AND WITH LOWER AMOUNTS OF WATER IN PREMIXING AND MINIMUM PREMIXING TIME

[Tar sands contained 7 wt. percent water, 13 wt. percent oil]

| Process                                   | Present Invention | Sand Reduction <sup>3</sup> |
|-------------------------------------------|-------------------|-----------------------------|
| Temperature, ° F.                         | 45                | 70                          |
| Premixing Time, Minutes                   | 0.5               | 5                           |
| Premixing Water, Wt. percent <sup>1</sup> | 30                | 75                          |
| Sand Removed, Wt. percent <sup>2</sup>    | 66                | 80                          |
| Oil Recovery, Wt. percent                 | 90                | 88                          |

<sup>1</sup> On tar sands (dry basis).

<sup>2</sup> Also contains oil not recovered in oil phase.

<sup>3</sup> Use of mechanical separation at atmospheric pressure.

From the above it is apparent that a better oil recovery is secured in a shorter time period when utilizing a vacuum separation technique.

EXAMPLE 3

In operation A, a mixing time of one minute was employed with a pressure of 200 mm. of mercury absolute. Under these conditions, about 65% of the sand was removed wherein the oil phase comprised 45% of oil.

In a similar Operation B, atmospheric pressure was employed and a mixing time of 5 minutes utilized. Under these conditions, about 50% of the sand was removed wherein the oil phase comprised about 33%. Thus, from the above it is apparent that the use of vacuum increases substantially the extent to which oil may be recovered.

The pressure utilized is below atmospheric, preferably in the range from 50 to 200 mm. of mercury absolute. In accordance with the present operation, the temperature may be atmospheric or may be in the range from 32 to 160° F.

It is felt that the desirable results of the present invention are secured due to the fact that the excess void volume in the tar sands that is not filled with oil and water is filled with gas. Some of the gas was dissolved in the oil. The presence of this gas in the tar sands is made to effect separation of an oil phase from sand in water at low temperatures.

What is claimed is:

1. Improved process for producing enriched bitumen tar sands from natural tar sands which comprises adding a fluid comprising water to natural sands and subject-

ing the mixture to a mixing-shearing action at a temperature in the range from about 50° F. to about 90° F., thereafter subjecting the mixture to a vacuum in the range from about 50 to 200 mm. of mercury absolute, and at a temperature in the range from about 32° F. to about 160° F. wherein substantially bitumen-free sands separate from enriched bitumen sands, thereafter separating said enriched bitumen sands from the substantially bitumen-free sands.

2. Process as defined by claim 1 wherein about 40% to 500% by weight, based upon dry bitumen sands, of water is added to said natural sands.

3. Process as defined by claim 2 wherein the temperature is maintained in the range from about 32° to about 110° F.

4. Process as defined by claim 2 wherein the quantity of water added is in the range from about 40% to about 150%.

5. Process as defined by claim 1 wherein the connate water content of said natural sands is from about 4% to 12%.

References Cited in the file of this patent

UNITED STATES PATENTS

|           |         |       |              |
|-----------|---------|-------|--------------|
| 1,396,173 | Fenton  | ----- | Nov. 8, 1921 |
| 2,825,677 | Coulson | ----- | Mar. 4, 1958 |

FOREIGN PATENTS

|    |         |        |       |               |
|----|---------|--------|-------|---------------|
| 30 | 523,067 | Canada | ----- | Mar. 20, 1956 |
|----|---------|--------|-------|---------------|